# EUROPEAN PATENT SPECIFICATION

(11) **EP 0 718 060 B1**
(45) Date of publication and mention of the grant of the patent: **10.02.1999**
(21) Application number: 95890217.3
(22) Date of filing: 12.12.1995
(51) Int. Cl.: B22D 19/14

(54) **Method and apparatus for producing a composite of particulate inorganic material and metal**
Verfahren und Vorrichtung zum Herstellen eines Verbundkörpers aus anorganischen Teilchen und Metall
Procédé et appareil pour la fabrication d'un composite à partir de particules inorganiques et de métal

(30) Priority: 22.12.1994 JP 320967/94; 02.03.1995 JP 42954/95; 02.03.1995 JP 42955/95; 15.05.1995 JP 116155/95
(43) Date of publication of application: 26.06.1996
(73) Proprietor: SUGITANI KINZOKU KOGYO KABUSHIKI KAISHA, Tokyo (JP); TOYO ALUMINIUM KABUSHIKI KAISHA, Osaka-shi Osaka-fu (JP)
(72) Inventor: Sugitani, Nobuhiro, c/o Sugitani Kinzoku Kogyo, Tokyo (JP)
(74) Representative: Krause, Walter, Dr. Dipl.-Ing.

(56) References cited:
- EP-A- 0 409 197
- GB-A- 1 275 518
- GB-A- 1 379 157
- US-A- 3 110 939
- US-A- 3 862 657
- US-A- 3 902 861
- US-A- 5 259 435

## Description

The present invention relates to a method for producing a composite product of an inorganic material and a metal and to an apparatus therefor.

For utilizing a hollow spherical particulate material, such as a calcined natural glass sand (Shirasu-balloons), for producing boards and blocks, a process is necessary for shaping (molding) it, while bonding the particles using a binding material. As the binding material, for example, resins, cements and sodium silicates have found their application therefor. Use of resins will result in a reduction of non-inflammability of the product, while use of cements may impair the contemplated light-weighing property and processibility of the product and use of sodium silicates may bring about inferior strength and lower processibility of the product.

A technique of producing composite boards has been known (Japanese Patent Application No.320967/1994), which comprises charging a mold cavity in a form of a plate with a hollow spherical particulate material and filling up the interstices of the charged particles with a molten metal, such as aluminum, to be used as the binding material, by impressing the molten metal into the mold cavity under a pneumatic pressure to soak the charged hollow particulate material. This technique has, however, defects that the dimensions of the composite board to be produced are limited to the range in which the flowability of the molten metal for soaking the hollow particles in the mold cavity can be maintained and that there is a large irregularity in the degree of filling up of the particle interstices with the metal over the product board, so that, even approximately, a homogeneous filling up and, therefore, uniformity of the material properties of the product board, cannot be achieved. These defects become increased when the board has greater extension or is thinner. For these reasons, this technique has not been in practice for the production of boards.

Processes of prior art for continuous production of uniform composites of inorganic material and metal are reviewed in our prior patent application (Japanese Patent Application No. 320967/1994, see above). A continuous production of boards may permit to expect a reduction in the production cost due to the high productivity, nevertheless there is a limitation in the design of the ornamental surface profile pattern on the board required for commercializing such boards. Thus, it is not able to produce a composite board having a surface profile of, for example, an undercut with a projection protruding rectangularly to the direction of sliding of the composite board along the inside face of the metal mold upon the production thereof. While it may be considered that a surface profile can be brought about by a roller embossing or a plate embossing after the composite board has been molded, such a measure may deteriorate the ornamental effect of the composite board due to the possible break down of the hollow particles of the inorganic material upon the embossing, since these hollow particles appear even within a quite shallow depth in the skin layer of the composite. For these reasons, the surface profile patterns achieved by the conventional continuous production techniques are limited to those in which the embossing patterns are quite shallow, e.g., hair-thick lines and the like, and run parallel with a constant width only in the direction of sliding of the composite board performed in the production thereof.

For producing a board or a block from hollow particulate material, the particles must be bonded rigidly together by, for example, using a binder. For such a binder, resins, cements, sodium silicates and others are used. Use of a synthetic resin for such a binder will result in a poor non-inflammability of the product. Use of cement will lead to a heavy-weighing product with poor processibility and use of sodium silicates brings about a product with lower strength and inferior processibility.

A technique has been known for producing a composite product from a hollow particulate material, which comprises filling up a plate-shaped mold cavity of a metal mold with the hollow particulate material and injecting therein a molten metal, such as aluminum, by impressing it by a pneumatic or a mechanical means to penetrate through the interstices between the particles, in order to bind the particles rigidly with each other by the metal as a medium for binding the particles.

This technique can only be applied to the case where the thickness of the product board allows a free flow of the molten metal to penetrate into the interstices between the particles. Thus, an allowable charging ratio of the molten metal to the particulate material, namely, a permissible uniformity in the material properties of the product composite can only difficulty be achieved.

The difficulties of the prior techniques as given above become more and more larger for products of greater size and lower thickness. For this reason, these techniques are still not in practical use for the production of composite board.

A technique has also been contrived, in which a molten metal is injected into a horizontally laying plate-shaped aggregation of a hollow particulate material in a horizontal mold from above to produce a composite impregnated with the metal. Here, the mold is provided at a portion thereof with a preheater to preheat the plate-shaped aggregation. However, due to the relationship between the geometry of the mold and the possible sliding velocity of the plate-shaped aggregation, it is difficult to choose a high preheating temperature of the aggregation of the particulate material. If the preheating temperature is lower, it is necessary to increase the pressure for injecting the molten metal into the aggregation in order to attain penetration into the interstices between the particles. This pressure calculates to be doubled as compared with the case of bilateral injection of the molten metal, since the penetration depth is doubled. If the injecting pressure is increased, the proportion of collapse of the hollow particles due to compression increases, resulting in an increase in the apparent density of the composite board obtained. A higher injecting pressure brings about a further defective effect of necessitating an increase in the strength of the molten metal storage vessel. A disadvantageous measure may be necessary for evading these defective effects, for example, by incorporating a greater heat source, in order to attain a prompt preheating of the hollow particulate inorganic material.

Various processes have been contrived for producing a composite of metal and hollow particles of inorganic material and some have found their practical applications. All of these prior processes are fundamentally based on the principle of compressingly impregnating the particles with a molten metal in a static condition. The compressive impregnation becomes more difficult, as the thickness of the particle layer increases and the path for the penetration of the molten metal becomes longer. A principal cause of such increase in the difficulty of impregnation may be the circumstances that the stream of the molten metal upon penetration into the aggregation of the particles on passing through the quite narrow interstices between the particles will be branched into thin streamlets of very small diameters which may be liable to a rapid quench and solidification, losing thus rapidly their fluidity and blocking up the flow. If this difficulty is overcome by forcing the molten metal to penetrate the aggregation of the particles by impressing it into the interstices between the particles, some bulky streams of the molten metal will appear up to some depth by wedging the hollow particles away, before they branch into dendritic very thin streamlets. Within the bulky stream, the hollow particles may be collapsed and the molten metal fills up the particle inside to deteriorate the characteristic feature of light-weighing of the composite and there is a large local inequality in the material properties between the portion of the bulky stream and the portion of the dendritic streamlets. In order to obviate these disadvantages, a new technique was proposed and a corresponding patent application was made (Japanese Patent Application Ser. No. 320967/1994), in which a molten metal is injected into a board-like aggregation of the hollow particulate inorganic material held in the mold cavity, through perforations of a perforated plate which covers only a restricted area of one side face of the mold cavity, by pneumatically impressing the molten metal with a relatively low compressive force (1.5 - 2.5 kgf/cm²) so as to attain the penetration of the molten metal in the direction of thickness of the board in which the path of penetration is at the smallest. This technique has been proven experimentally to be a process for producing a composite board of a metal and a hollow particulate inorganic material exhibiting the lowermost local inequality in the material properties. This material property inequality which is the principal disadvantage of this technique increases, however, in proportion to the thickness of the bulk of aggregation for a composite product of a thick aggregation, such as a block, cylinder of larger diameter or the like, since the molten metal permeates through the interstices between the particles in the aggregation. It has therefore been expected to provide a method for producing composite products of a metal and a hollow particulate inorganic material with greater bulk thickness, by which such a local inequality in the material properties of the resulting composite product is minimized.

In GB-A-1 275 518 it is described that a molten metal is introduced into a pipe of an inorganic high melting light-weight material. However, a concrete method of introducing molten metal is not disclosed in this reference, and invention of this application, in which molten metal is injected into the mold cavity through a perforated refractory plate having many small perforations, is completely different from this reference.

US-A-3 862 657 discloses that metal and additives 20 are mixed and introduced into a hollow mold compartment. However, in the present invention, molten metal is injected into the mold caving through the molten metal permeable perforated or porous part of the passage mold, which is completely different from this reference.

In US-A-5 259 435 is described that fine-meshed stainless steel wire netting is placed over the layer of carbon pellets in order to reduce composite material block. However, in the present invention, molten metal is injected into the mold caving through the perforated or porous part to cause the molten metal to penetrate the aggregation of the inorganic material through the interstices between the particles of the aggregation in order to solidify into the extended product.

The first object of the present invention is to obviate the above-mentioned disadvantages of the prior art processes and to provide novel processes and novel apparatuses for producing an extended relatively thin product of a composite of a metal and a hollow particulate inorganic material exhibiting a lower local inequality in the material properties of the resulting product.

The second object of the present invention is to provide another novel process and a novel apparatus adapted for producing an extended product of a composite of a metal and a hollow particulate inorganic material having a voluntarily designed surface relief pattern and exhibiting a lower local inequality in the material properties of the resulting product, in a continuous manner without limitation of the extension of the resulting composite product.

The third object of the present invention is to provide a further novel process and a novel apparatus for producing an extended product of a composite of a metal and a hollow particulate inorganic material in a form of a board, cylinder or block, in a continuous way with continuous charging of the hollow particulate inorganic material to a stationary passing mold.

The fourth object of the present invention is to obviate the disadvantages of the prior art processes and to provide a still further novel process and a novel apparatus adapted for producing an extended product of a composite of a metal and a hollow particulate inorganic material having a greater bulk thickness and exhibiting a lower local inequality in the material properties of the resulting product, in a continuous way without limitation in the extension of the product using a high-temperature mixer extruder.

The invention is defined in claims 1, 3, 4 and 5. Preferred embodiments are defined in claims 2 and 6-21.

More specifically, the first object of the present invention is attained, in the first place, by a process for producing an extended relatively thin composite product of a metal and a hollow particulate inorganic material using a mold assembly which is constituted essentially of
a mold enclosing a mold cavity of a geometry corresponding to the extended product, a means for charging the mold cavity with the hollow particulate inorganic material, a storage vessel for storing the molten metal, a molten metal permeable perforated or porous refractory plate located on one side of the extension of the mold cavity and adjoining the molten metal in said storage vessel and a means for taking the molded composite product out of the mold cavity,
said process comprising the process steps of
filling up the mold cavity of the mold with the hollow particulate inorganic material to build up an aggregation of the particulate inorganic material in a form corresponding to the mold cavity,
injecting the molten metal into the aggregation of the particulate inorganic material in the mold cavity through the molten metal permeable perforated or porous plate to cause the molten metal to penetrate into the interstices between the particles in the aggregation by pneumatically impressing the molten metal in the molten metal storage vessel,
permitting the resulting product composed of the aggregation of the particulate inorganic material and the molten metal penetrated said aggregate to solidify into the extended product of the composite of metal and hollow particulate inorganic material and
taking the solidified composite product out of the mold cavity.

The above-mentioned first object of the present invention is also achieved, in the second place, by a process for producing an extended relatively thin composite product of a metal and a hollow particulate inorganic material using a mold assembly which is constituted essentially of
a mold enclosing a mold cavity subdivided at an equal interval into an entrance section, a central section and an exit section each having the same geometry corresponding to the extended product; a means for charging the entrance section of the mold cavity with the hollow particulate inorganic material; a means for forwarding the resulting aggregation slidingly stepwise successively from the entrance section to the central and the exit sections and, finally, to the outside of the mold; a storage vessel for storing the molten metal; a molten metal permeable perforated or porous refractory plate located on one side of the extension of the mold cavity and adjoining to the molten metal in said storage vessel; and a means for taking the molded composite product out of the mold,
said process comprising repeating the process steps of
filling up the entrance section of the mold cavity with the hollow particulate inorganic material to build up an aggregation of the particulate inorganic material therein in a form corresponding to the mold cavity of the entrance section,
forwarding this aggregation slidingly stepwise, first, to the central section of the mold cavity,
injecting the molten metal into the particle aggregation in the central section of the mold cavity through the molten metal permeable perforated or porous plate to cause the molten metal to penetrate the aggregation through the interstices between the particles of said aggregation of the hollow particulate inorganic material by pneumatically impressing the molten metal in the molten metal storage vessel, while re-filling the now vacant entrance section with fresh hollow particulate inorganic material,
forwarding, then, the aggregation found in the central section and now impregnated with the molten metal slidingly stepwise to the exit section of the mold cavity, while repeating the above re-filling and injecting steps,
cooling, thereafter, the resulting molded product in the exit section of the mold cavity to solidify it into the extended product of the composite of metal and hollow particulate inorganic material,
forwarding, then, the aggregations in the three sections slidingly stepwise further to move the solidified product to the outside of the mold, while repeating the above process steps, and
taking the finished molded composite product out of the mold assembly in the discharge station.

The above-mentioned first object of the present invention is also achieved, in the third place, by a novel apparatus for producing an extended relatively thin composite product of a metal and a hollow particulate inorganic material, comprising a mold assembly which comprises
a mold enclosing a mold cavity of a geometry corresponding to that of the extended composite product,
a means for charging the mold cavity with the hollow particulate inorganic material to fill it up and to shape it into an aggregation of the hollow particulate inorganic material,
a means for slidingly forwarding the aggregation of the hollow particulate inorganic material from the charging end to a discharge station of the mold assembly,
a storage vessel for storing the molten metal and adapted to be pneumatically impressed for effecting injection of the molten metal into the mold cavity,
a molten metal permeable perforated or porous refractory plate for injecting the molten metal there-through into the aggregation of the hollow particulate inorganic material in the mold cavity, located on one side of the extension of the mold cavity and adjoining to the molten metal in said storage vessel, with its perforations or pore channels being distributed over the plate and each having a diameter adapted to permit the molten metal to be injected therethrough into the aggregation upon the pneumatic impression but not adapted to permit the hollow particles of the inorganic material in the aggregation to intrude into the molten metal in said storage vessel and
a means for taking the molded composite product out of the mold cavity at the discharge station.

The above-mentioned first object of the present invention is also achieved furthermore, in the fourth place, by a novel apparatus for producing an extended relatively thin composite product of a metal and a hollow particulate inorganic material successively, comprising a mold assembly which comprises
a mold enclosing a mold cavity subdivided at an equal interval into an entrance section, a central section and an exit section each having the same profile geometry as that of the extended product,
a means for charging the entrance section of the mold cavity with the hollow particulate inorganic material to fill it up and to build up an aggregation of the hollow particulate inorganic material therein,
a means for slidingly forwarding stepwise the aggregation of the hollow particulate inorganic material in the entrance section successively to the central and the exit sections of the mold cavity and, finally, to the discharge station of the mold assembly,
a storage vessel for storing the molten metal, located adjacent the mold cavity and adapted to be pneumatically impressed for effecting injection of the molten metal into the central section of the mold cavity,
a molten metal permeable perforated or porous refractory plate for injecting the molten metal therethrough into the aggregation of the hollow particulate inorganic material in the mold cavity, disposed on one side of the extension of the mold cavity and adjoining to the molten metal in said storage vessel, with its perforations or pore channels being distributed over the plate and each having a diameter adapted to permit the molten metal to be injected therethrough into the aggregation upon the pneumatic impression but not adapted to permit the hollow particles of the inorganic material in the aggregation to intrude into the molten metal in said storage vessel, and
a means for taking the molded composite product out of the mold cavity at the discharge station.

More specifically, the second object of the present invention is attained by a novel process for producing an extended relatively thin product of a composite of a metal and a hollow particulate inorganic material having a voluntarily designed surface relief pattern successively using a mold assembly constituted essentially of
mold elements enclosing a mold cavity having a profile geometry corresponding to that of the extended product of the composite and composed of a plurality of mold bottom segments slidably movable on a mold bed and on inlet side and outlet side mold guide, respectively, and a molten metal permeable stationary perforated or porous refractory plate; a means for charging the mold cavity with said hollow particulate inorganic material; and a storage vessel for storing the molten metal, with its bottom being constituted of said molten metal permeable perforated or porous refractory plate,
said process comprising, under repetition, the process steps of
laying the mold bottom segments serially on the mold bed to form a mold bed train,
filling up the mold cavity on the mold bottom segment at the mold inlet with the hollow particulate inorganic material to build up an aggregation of the particulate inorganic material in a form corresponding to the mold cavity,
forwarding the mold bottom train slidingly on a mold guide way and on the mold bed together with the aggregation of the hollow particulate inorganic material towards the mold outlet,
injecting the molten metal into the mold cavity through the molten metal permeable perforated or porous refractory plate constituting the bottom of the molten metal storage vessel by pneumatically impressing the molten metal in the molten metal storage vessel to cause the molten metal to penetrate the aggregation through the interstices between the particles of the aggregation,
taking out the molded extended composite product impregnated with the molten metal from the mold bottom segment left the mold as the mold bottom moves on, and
removing the foremost mold bottom segment now freed from the molded composite product at the mold outlet end from the outlet side mold guide way and laying it again on the inlet side mold guide way to supplement the mold bottom train.

The second object of the present invention is also attained by a novel apparatus for producing an extended relatively thin product of a composite of a metal and a hollow particulate inorganic material having a voluntarily designed surface relief pattern successively, comprising a mold assembly constituted essentially of
mold elements enclosing a mold cavity having a profile geometry corresponding to that of the extended product of the composite and composed of a plurality of mold bottom segments, which are arranged in a tight but separable fitting with each other to build up a trough-formed mold bottom train slidably movable on a mold guide way and on a mold bed and each of which has a voluntarily designed surface relief pattern on the upper face thereof, and a molten metal permeable stationary perforated or porous refractory plate defining the upper limit of the mold cavity,
a means for charging the mold cavity with said hollow particulate inorganic material to build up an aggregation of the hollow particles of the inorganic material in the mold cavity,
a means for forwarding the mold bottom train slidingly on the mold guide way and on the mold bed together with said aggregation of the
particulate inorganic material carried thereon, from the inlet side to the outlet side of the mold assembly,

a storage vessel for storing the molten metal disposed on the molten metal permeable stationary perforated or porous refractory plate and adapted to be pneumatically impressed for effecting injection of the molten metal into the mold cavity charged with the aggregation of the hollow particulate inorganic material through the molten metal permeable stationary perforated or porous refractory plate, said perforations or pore channels being distributed over the plate and each having a diameter adapted to permit the molten metal to be injected therethrough into the aggregation of the particles of the inorganic material upon the pneumatic impression of the molten metal but not adapted to permit the particles of the inorganic material to intrude into the molten metal in said storage vessel, and

a means for taking out the molded extended composite product from the mold bottom segment moved and left the mold cavity.

More specifically, the third object of the present invention is attained by a novel process for producing an extended product of a composite of a metal and a hollow particulate inorganic material in a form of a board, cylinder or block, in a continuous way with continuous charging of the hollow particulate inorganic material using a mold assembly constituted essentially of
a stationary passage mold enclosing an extended mold cavity and subdivided into a preheating zone accommodated in a molten metal storage vessel, a molten metal injection zone of molten metal permeable perforated or porous part, with its perforations or pore channels being distributed over this zone, immersed in the molten metal for permitting injection of the molten metal into the mold cavity therethrough and a cooling zone in the mold exit end portion; an assembly for charging the mold cavity with said hollow particulate inorganic material at the mold inlet; and a towing means for pulling down the resulting extended composite product to be discharged out of the mold,
said process comprising the process steps of
charging the mold cavity at the mold inlet with the hollow particulate inorganic material to build up an aggregation of the hollow particulate inorganic material in a cross-sectional profile corresponding to that of the mold cavity,
forwarding the resulting aggregation of the particulate inorganic material slidingly towards the mold exit by the action of the towing means,
injecting the molten metal into the mold cavity through the molten metal permeable perforated or porous part of the passage mold to cause the molten metal to penetrate the aggregation of the particulate inorganic material though the interstices between the particles of the aggregation by a static pressure head of the molten metal in the molten metal storage vessel and, if necessary, under a pneumatic pressure control in the molten metal storage vessel,
cooling the aggregate impregnated with the molten metal in the cooling zone of the stationary mold to solidify it and
taking the so-solidified extended composite product out of the mold under the use of the towing means.

The third object of the present invention is also attained by a novel apparatus for producing an extended product of a composite of a metal and a hollow particulate inorganic material in a form of a board, cylinder or block, in a continuous way with continuous charging of the hollow particulate inorganic material, said apparatus comprising a mold assembly which comprises
an extended stationary passage mold enclosing an extended mold cavity having a cross-sectional profile geometry corresponding to that of the extended product of the composite passing therethrough and subdivided into a preheating zone accommodated in a molten metal storage vessel, a molten metal injection zone of molten metal permeable perforated or porous part, with its perforations or porechannels being distributed over this zone, immersed in the molten metal for permitting injection of the molten metal into the mold cavity therethrough provided with perforations distributed over this zone and a cooling zone in the mold outlet end portion for cooling and solidifying the molded product in the mold cavity,
an assembly for charging the mold cavity with the hollow particulate inorganic material at the mold inlet to build up an aggregation of the particulate inorganic material in the mold cavity and
a towing means for pulling out the resulting extended composite product from the mold cavity, disposed subsequent to the mold outlet.

More specifically, the fourth object of the present invention is attained by a novel process for producing an extended shaped product of a composite of a metal and a hollow particulate inorganic material having a relatively greater bulk thickness in a form of, such as, a board, cylinder, block or so on, in a continuous way using a molding apparatus constituted essentially of
a high temperature mixer extruder for mixing the hollow particulate inorganic material with the molten metal and extruding the resulting mixture from an extruding nozzle; a means for supplying the mixer extruder with the hollow particulate inorganic material; a means for supplying mixer extruder with the molten metal; and a shaping unit for shaping the mixture extruded from the mixer extruder into the final shaped product of the composite,
said process comprising the process steps of
mixing the hollow particulate inorganic material and the molten metal on the mixer extruder,
extruding the resulting mixture into the shaping unit to shape it into a shaped green product,
cooling the shaped green product to solidify into the final product and
taking this product out of the shaping unit.

The fourth object of the present invention is attained also by a novel apparatus for producing an extended shaped product of a composite of a metal and a hollow particulate inorganic material having a relatively greater bulk thickness in a form of, such as, a board, cylinder, block or so on, in a continuous way, comprising
a molten metal storage vessel,
a high-temperature mixer extruder for mixing the particulate inorganic material with the molten metal and for extruding the resulting mixture from an extruding nozzle, said mixer extruder having a refractory casing cylinder capable of being heated to a temperature above the solidifying point of the molten metal,
a means for supplying the mixer extruder with the hollow particulate inorganic material,
a means for supplying the mixer extruder with the molten metal and
a shaping unit for shaping the mixture extruded from the mixer extruder into the final shaped product of the composite.

Fig. 1 shows the first embodiment of the apparatus for producing a composite product of a particulate inorganic material and a metal according to the present invention in a vertical section.
Fig. 2 is a partly sectioned side view of the principal portion of the apparatus of Fig. 1.
Figs. 3(a) and 3(b) show each the essential portion for injecting molten metal into the mold cavity filled with an aggregation of the particulate inorganic material in an enlarged vertical section, wherein Fig. 3(a) shows the state during the molten metal injection and Fig. 3(b) shows the state upon slidingly forwarding the resulting composite after the metal impregnation.
Fig. 4 shows a part of the horizontal section of the perforated plate along the line IV-IV of Fig. 3 in an enlarged view.
Fig. 5 shows the essential part of the second embodiment of the apparatus for producing a composite product of a hollow particulate inorganic material and a metal according to the present invention in a partly sectioned front view.
Fig. 6 is a side view of the apparatus of Fig. 5 in the central vertical section.
Fig. 7 shows the third embodiment of the apparatus for producing a composite product of a particulate inorganic material and a metal according to the present invention in a vertical section.
Fig. 8 shows the state of charging of the mold cavity with the particulate inorganic material and injection of molten metal thereinto in the apparatus of Fig. 7 in a partial enlargement.
Fig. 9 shows the fourth embodiment of the apparatus for producing a composite product of a particulate inorganic material and a metal according to the present invention in a vertical side section.

First, the process for producing an extended composite product of a particulate inorganic material and a metal according to the present invention is described in detail, in particular, for the cases of successive production of the composite product using a horizontally laid molding assembly, based on the first embodiment thereof with reference to Figs. 1 to 4.

The entire apparatus can be seen from Figs. 1 and 2, in which 1 is a gas-tight lid operating cylinder, 2 is a gas-tight lid, 3 denotes a gas-tight lid fixing member, 4 designates a particulate inorganic material hopper which is supplied with the hollow particulate inorganic material by, for example, a belt conveyer and 5 is a storage vessel (crucible furnace) for storing the molten metal. The essential portion of the apparatus where the molten metal is injected into the aggregation of the particulate inorganic material is indicated by 6. The hopper 4 adjoins at its bottom to the inlet of the mold cavity via an opening permitted to open and close voluntarily.

In the portion 6, the crucible furnace 5 is surrounded by a heat insulator wall 7 constituted of refractory bricks and a binding plaster for preventing dissipation of heat. In the crucible 8 of the crucible furnace 5, a molten metal 10 is stored. The molten metal 10 is pneumatically impressed, as shown by the arrows 9. The gas-tight lid 2 is brought down by an action of the gas-tight lid operating cylinder 1 and closes the furnace 5. The crucible 8 is sealed tightly by means of a lid fixing member 3, whereupon the gas space of the crucible is supplied with a compressed air through an air supply path provided in the gas-tight lid 2 to impress the molten metal 10. An operator 11 is disposed adjacent the above-mentioned portion 6 for operating a pusher plate 14 for slidingly forwarding the aggregation of the hollow particulate inorganic material and serving also as a stopper for the molten metal in the mold cavity 13'' in the mold 13. The metal mold 13 is arranged beneath the crucible 8 and has, on its upper wall, a thin-walled area 13' which is provided with many perforations 12 distributed over this area at a definite interval so as to permit a uniform injection of the molten metal over this area into the aggregation 16 in the mold cavity 13'' in order to prevent unequal local concentration of the hollow particles in the aggregation 16 upon the injection of the molten metal.

In an alternative embodiment, the thin-walled area 13' is made of a molten metal permeable porous refractory material, such as unglazed pottery, with the pore channels for permeation of the molten metal having diameters adapted to permit the molten metal to be injected therethrough into the aggregation of the hollow particles of the inorganic material upon the pneumatic impression but not adapted to permit these hollow particles to intrude into the molten metal in the storage vessel.

The mold cavity 13'' is defined by surfaces exhibiting sufficient resistances to heat, corrosion and wear and a self-lubricating property to leave a space of the sectional geometry corresponding to that of the composite product 17 to be molded and is filled with the hollow particulate inorganic material to build up an aggregation. To fill up this mold cavity 13'' with a predetermined amount of the hollow particulate inorganicmaterial, a slidable pusher plate 14 is used, which is operated by the operator 11.

In the mold cavity 13'', a composite product 17 of a hollow particulate inorganic material and a metal is molded. For taking the composite product 17 out of the mold, a drawer plate 21 having formed at its drawn end one or more dovetail recesses 18 is employed. The molded composite product 17 solidifies in the dovetail recess 18 and forms a disengageable but rigid joint therewith for slidingly drawing out the solidified product. The drawer plate 21 is operated by an operator 20 for operating the drawer plate 21. After the molded composite product 17 has been solidified in the mold cavity, it is slidingly forwarded by a combined operation of the pusher plate 14 and the drawer plate 21 by their operators 11 and 20 to a discharge station outside the mold, where it is removed from the dovetail recess and is taken up.

The manner of operation of the mold assembly of the first embodiment of the present invention is as follows.

The gas-tight lid 2 is settled in position by actuating the gas-tight lid operating cylinder 1 located above the molten metal storage vessel 5 to seal the crucible 8 thereof so as to permit to pressurize the gas space thereof. For preventing leakage of the compressed air, the gas-tight lid 2 is fixed to the storage vessel 5 by fixing members 3. After the lid 2 has been fixed, a compressed air is supplied to the gas space of the storage vessel 5 via an air path formed in the lid 2 to cause the molten metal 10 to be impressed pneumatically (9). The temperature of the molten metal stored in the crucible 8 is maintained by a heater 22 at a predetermined value. The temperature of the molten metal 10 and that of the surface thereof are detected by corresponding thermosensors (not shown). A hollow particulate inorganic material is introduced into the mold cavity 13'' of the mold 13 from the hopper 4 and is guided through a preheating zone to a metal injection zone by the aid of the pusher plate 14, before it is compacted into an aggregation 16 of the particles [See Fig. 3(a)]. By the pneumatic impression (9) of the molten metal 10, it is introduced into the aggregation 16 of the particulate material through the perforations 12 formed in the thin-walled area 13' of the upper wall of the mold 13. After the aggregation 16 of the particulate material has been impregnated by the molten metal injected therein, the metal is cooled and solidified. Here, any noticeable inequality in the distribution of the mixing ratio of the metal to the particulate material is avoided, since the molten metal is injected from a large number of small perforations 12 and, therefore, under a uniform distribution over a wide area into the aggregation 16. Upon injection of the molten metal into the aggregation, the light-weighing hollow particles will tend to float up in the heavy-weighing molten metal. Nevertheless, the hollow particles will be caught by each other within the narrow stream in the thin perforation 12 and cannot float up before the aggregation has been impregnated with the molten metal.

The aggregation 16 is slidingly forwarded stepwise, as shown by the arrow 19, in the mold cavity at a predetermined sliding interval by the combined operation of the means (11, 20) for slidingly forwarding the aggregation, while being impregnated with the molten metal, and is caused to solidify as a composite molded product 17 after having passed the mold outlet. The extended composite molded product 17 is guided by combined operation of the operators 11 and 20 onto a conveyer before it reaches the discharge station, where the molded composite product is taken up by disengaging the dovetail joint by sliding the molded product 17 and the drawer plate 21 in vertical direction to each other.

The stroke of the stepwise forwarding of the extended molded product corresponds to the longitudinal length of the aggregation to be impregnated with the molten metal in a single step [See Fig(b)]. The reciprocating motion of the operator 11 for the pusher plate 14 agrees completely with that of the operator 20 for the drawer plate 21 in respect of the stroke and timing. In each cycle of this synchronized motion, the impregnation of the aggregation with the molten metal through the perforations 12 by a pneumatic impression is repeated. Replenishment of the mold cavity with the hollow particulate inorganic material is effected on each retrogression stroke of the operator 11 for the pusher plate 14 by regulating the discharge gate of the hopper 4 to open. Replenishment of the storage vessel 5 with the molten metal is effected upon detection of arrival of the surface of the melt in the storage vessel 5 at a predetermined level by a melt level sensor disposed in the crucible 8, by which an electric signal is given out to cease the operations of the operators 11 and 20 temporarily and to exhaust the compressed air in the gas space of the storage vessel 5 out of it, whereupon the gas-tight lid 2 is lifted by operating the gas-tight lid operating cylinder 1 for starting the replenishment of the molten metal. While it is preferable to operate the above-described mold assembly continuously without cessation, the assembly may eventually be forced to be brought to out-of-operation for some periods of times by whatever reason. In this case, the operation of the mold assembly is continued until the molten metal in the crucible and in the mold cavity has been emptied completely, before the operation is stopped. For starting the operation again, the mold cavity is cleaned from the residual particulate material and is then filled with the fresh hollow particulate material under resetting of the pusher plate 14 and the drawer plate 21 at the start position, whereupon the crucible 8 is re-filled with the molten metal by pursuing the procedures as in the starting of the mold assembly, before the operation is started again.

The particulate inorganic material to be used according to the present invention is a hollow spherical particulate inorganic material, such as that obtained by calcinating the naturally occurring fine particulate Shirasu (a kind of volcano ejecta deposit) existing as one of abundant resources, or foamed glass beads. It has a bulk density of 0.3 to 0.4 g/cm² and a particle size of 0.3 to 2.5 mm.

Now, the process for producing an extended composite product of a particulate inorganic material and a metal according to the present invention is described for the case of continuous production of the composite product using a horizontally laid mold assembly, based on the second embodiment thereof with reference to Figs. 5 and 6.

In the apparatus as shown in Figs. 5 and 6, a gas-tight lid operating cylinder 31 is arranged above a molten metal storage vessel 35 and is operable so as to impress a gas-tight lid 33 onto the rim ridge of a flange member 32 of the storage vessel 35 to realize a gas-tight seal of the storage vessel 35. On both sides of the gas-tight lid 33 are disposed each, opposingly to each other, a horizontal piston/cylinder arrangement 34 by which the lid 33 can be maintained under impression thereof onto the flange member 32. Around the storage vessel 35 is arranged a heater 36 and, outside thereof, a layer of a heat insulator 37. Outside the heat insulator, a pile of refractory bricks 38 surrounds the storage vessel assembly. The storage vessel 35 stores a molten metal 39.

Beneath the storage vessel 35, a horizontal mold is disposed which is composed of mold elements. The mold elements are composed of, on the one hand, a plurality of trough-formed mold bottom segments 44 connected to each other to form a mold bottom train slidably movable on a mold bed 41 and, on the other hand, a stationary perforated refractory plate 40 having many small perforations. The mold elements constitute a horizontal passage mold in the region beneath the stationary perforated refractory plate 40. The perforated refractory plate 40 is fitted to the open bottom of the molten metal storage vessel 35 so as to constitute a perforated bottom plate of the storage vessel 35 so that the perforations thereof permit the molten metal 39 to be injected into the mold cavity 45 of the mold therethrough. The perforated refractory plate 40 may be replaced by a molten metal permeable porous refractory plate, as explained in the first embodiment of the present invention hereinbefore. The mold bed 41 is supported on a stand 53 fixedly under an interposition of an insulator board 42. Each of the mold bottom segments 44 has the same geometry and profile and is provided on its upper face with a voluntarily designed (negative) surface relief pattern for imparting corresponding (positive) relief.

On the commencement of the molding operation using the above-described mold assembly, a solid dummy segment 43 having the same sectional contour geometry as the mold bottom segment is placed at the forehead of the train of the mold bottom segments 44 on the mold bed 41, in order to plug the perforations of the mold bottom segment to prevent free flowing down of the molten metal through them before the start of the molding. The solid dummy segment 43 can be forwarded slidingly on the mold bed 41 together with the succeeding mold bottom segments 44 and may have a voluntarily selected longitudinal length. The trailing end of the solid dummy segment 43 is tightly fitted to the front end of the forefront mold bottom segment 44 and, therefore, can slidably be forwarded on the mold bed 41 together with the subsequent mold bottom train. On forwarding the so-connected train of the solid dummy segment 43 and the following mold bottom segments 44 slidingly on the mold bed 41, the perforations in the stationary refractory plate 40 become open to the mold cavity above the succeeding mold bottom segment and the molten metal in the storage vessel 45 begins to spout into the mold cavity which has been filled with an aggregation of the hollow particulate inorganic material as described below. The solid dummy segment 43 is taken off from the mold bottom train after the dummy segment has reached a take-out station on the mold outlet side (the left side in Fig. 6).

The hollow particles of inorganic material supplied via an adequate means, such as a conveyer (not shown), are once stored in a hopper 46, from a gate opening of which they are introduced into the mold cavity 45 above the mold bottom segment 44 before it is forwarded to the position beneath the bottom of the molten.

The sliding movement of the mold bottom train is performed by means of a piston/cylinder arrangement 48. The piston rod thereof is provided at its terminal end with an engagement bracket supported on a wheeled support 49 movable in a guide groove 50 of a guide rail, with which the mold bottom train can be pushed slidingly forward (to the left of Fig. 6) on the inlet side guide way formed by guide rollers 51 and then on the mold bed 41 upon the forwarding stroke of the piston/cylinder arrangement 48. The mold bottom train is guided to an outlet side guide way formed by the guide rollers 51, after passing through the mold outlet. The guide rollers 51 are supported on a guide roller supporting bracket 52 supported on the stand 53.

In the production of a molded product of a composite of a metal and a hollow particulate inorganic material using the above-described mold assembly, as shown in Fig. 6, the hollow particulate inorganic material supplied via a suitable means, such as a belt conveyer (not shown) is once stored in a hopper 46, from which it is introduced into the mold cavity 45 above the mold bottom segment 44 before it is forwarded to the position beneath the bottom of the molten metal storage vessel 35. While the mold bottom train passes through the mold region beneath the stationary perforated refractory plate 40 at a constant velocity, the molten metal 39 in the molten metal storage vessel 35 is injected into the aggregation of the hollow particulate inorganic material formed in the extended mold cavity 45 on the mold bottom train. By impression of the molten metal 39 in the storage vessel 35 in a pneumatic way by, for example, supplying an inert gas or air to the gas space of the storage vessel 35, the injection of the molten metal through the fine perforations in the stationary refractory plate 40 is facilitated favorably, whereby a uniform composite product of the metal and the hollow particulate inorganic material is molded in a plate-like form with a voluntarily designed surface profile pattern. Thus, any contemplated voluntarily designed surface profile pattern of a definite size can be obtained.

Now, the process for producing a composite product of a particulate inorganic material and a metal according to the present invention is further described for the case of continuous production using a mold assembly provided with a stationary extended passage mold having many perforations and immersed in a molten metal storage vessel, based on the third embodiment thereof with reference to Figs. 7 and 8.

The mold assembly is provided on a stand (not shown) with a molten metal storage vessel 71, on which a hollow particulate inorganic material charger unit 64 provided with a charging screw driven by an electric motor 61 is mounted by a support. The screw shaft 63 of the screw is connected with the electric motor 61 disconnectably via a joint 62. The screw shaft 63 is supported ratably on the casing of the charger unit 64 by bearings 65 and 66 disposed at its upper and lower portions, respectively.

The charger unit 64 is provided, supported on the storage vessel 71, with a hopper 67 for supplying the hollow particulate inorganic material 68. The hollow particulate inorganic material 68 is guided by the screw into the inner chamber thereof and is forced by the screw into the inlet of the extended passage mold 69, which extends down vertically from the discharge end of the charger unit 64.

The passage mold 69 may be in a form of a flat conduit with a plate-formed internal passage way as the mold cavity or in a form of a tube with an internal passage way of a cylindrical, rectangular or polygonal cross-section as the mold cavity and is supported on the upper wall of the molten metal storage vessel 71 by a flange formed at the inlet thereof. The passage mold 69 is immersed in the molten metal 72 in the molten metal storage vessel 71 at the lower region provided with many small perforations and is supported at its lower end portion tightly in an opening penetrating the bottom wall of the vessel 71. Beneath the molten metal storage vessel 71 is arranged, surrounding the lower part of the extended passage mold 69, a cooling jacket 77, through which a cooling water is circulated by a circulation pump (not shown). Below the cooling jacket 77, a pair of guide rollers 76 are arranged, between which the cooled and solidified molded composite product discharged from the outlet of the extended passage mold 69 is pinched and towed downwards. The front end of the molded composite product which is discharged out of the mold upon the beginning of the molding is connected with a dummy plate (or dummy rod) 74 to assist towing down of the molded product.

The extended stationary vertical passage mold 69 is provided with many small perforations 69a in its lower region immersed in the molten metal 72. Instead of the perforations, this region may be made of a molten metal permeable porous refractory material, as explained in the first and the second embodiment of the present invention. The molten metal storage vessel 71 is provided on its ceiling wall with a dismountable gas-tight lid 75 and along its side or bottom wall with a heater means 73 embedded in the wall for maintaining the requisite temperature of the molten metal 72 stored therein.

By this molding apparatus, the hollow particulate inorganic material is supplied continuously to the extended vertical passage mold 69 from hopper 67 through the screw charger unit 64 by rotating the screw shaft 63 by the electric motor 61 via the disengageable joint 62 and is forced into the mold inlet through a conically converging guide horn of the charger unit 64. The hollow particulate inorganic material forced into the passage mold 69 by the screw builds up therein an aggregation of the particles, which is guided down by the wedging action by the screw charger together with a towing action by the pair of guide rollers 76 and reaches the heating zone surrounded by the molten metal 72, where the molten metal 72 is injected through the fine perforations distributed over this zone into the aggregation inside the mold cavity 70 of the mold 69. The molten metal injected into the aggregation of the hollow spherical particles penetrates through the intersices between the particles and fills up these interstices to form a composite mixture of the metal and the particulate inorganic material (See Fig. 8). This composite mixture descends within the mold cavity through the cooling zone thereof, where it is cooled and solidified by the cooling water 78 in the cooling jacket 77 into the molded composite product, which is towed down by the guide rollers 76. In Fig. 7, the molded composite mixture is shown in the mold cavity at a position at which it is brought into connection with the trailing end 79 of the dummy plate 74 inserted into the mold cavity.

finally, the process for producing an extended product of a composite of a metal and a particulate inorganic material according to the present invention is described for the case of continuous production of the composite product which has a relatively greater bulk thickness, such as a board, cylinder, block or so on, using a molding apparatus including a high-temperature mixer extruder, based on the fourth embodiment thereof with reference to Fig. 9.

The molding apparatus according to the fourth embodiment as shown in Fig. 9 is mounted on a stand 103 and includes a storage vessel 82 having a gas-tight lid 81 for storing a molten metal, such as aluminum etc. The gas-tight lid 81 can be assembled or disassembled by a lid assemblage piston/cylinder arrangement (not shown). For heating the molten metal at a temperature slightly above the melting point of the metal, a heating means 84 is installed in the molten metal storage vessel 82 under penetration through the gas-tight lid 81 and extending submerged under the molten metal layer 83. A thermosensor 85 is inserted in a protective sheath fixed arranged in the gas-tight lid 81 in a gas-tight fashion so as to submerge its top end beneath the level of the molten metal 83 for detecting the temperature of the molten metal 83 in the storage vessel 82. The molten metal storage vessel 82 communicates, via a graphite discharge socket 86 inserted in the bottom wall thereof, to a horizontally laid high-temperature mixer extruder of a screw conveyer-like construction constituted essentially of a screw 89 and a refractory casing cylinder 90 encasing the screw and made of, for example, graphite, so as to permit the molten metal to be introduced into the mixing space of the mixer extruder between the casing cylinder 90 and the screw 89. The high-temperature mixer extruder is supplied also with the hollow particulate inorganic material at a portion upstream the position where the grafite discharge socket 86 opens into the casing cylinder 90 of the mixer extruder. The molten metal and the hollow particulate inorganic material introduced into the high-temperature mixer extruder are mixed in the mixing space thereof by a kneading action caused by rotation of the screw 89.

Encased in a reinforcing steel sleeve, a heating means 88, such as a high-frequency coil, is arranged surrounding the refractory casing cylinder 90 for maintaining the temperature of the kneaded mixture within the casing cylinder 90 and is covered by a layer of heat insulator for preventing dissipation of the heat from the kneaded mixture, which is further covered by a coverage case 87.

The discharge end of the screw shaft is rotatably supported at the discharge end in a front end bearing 91 and at the opposing rear end in a rear end bearing 92, respectively. The front end and the rear end bearings are supported fixedly on the stand 103. The screw shaft is connected at its rear end, via a coupling 93 and a gearing, with a driving shaft of an electric motor 94 to permit a continuous operation of the screw 89.

The hollow particulate inorganic material is supplied to the high-temperature mixer extruder from a hopper 97 disposed above the mixer extruder at a portion upstream the supply inlet for the molten metal through a controllable gate. The hopper 97 is supplied with the hollow particulate inorganic material, such as "Shirasu balloons", which are obtained as a calcined product of a volcano ejecta deposit and have a bulk density of 0.3 - 0.5 g/ml³, from a preheating kiln (not shown) at a temperature of about 350 - 400 and is provided with an air-vibrator 95 for facilitating a smooth charging of the particulate material 96 into the mixer extruder and a preheater (not shown) for preheating the particulate material up to about 350 - 400 , before it is introduced into the mixer extruder.

The front bearing 91 for pivoting the discharge end of the screw shaft is provided with a plurality of openings for permitting extrusion of the kneaded mixture from the mixing space into a shaping unit 100 bodily connected with the mixer extruder. The shaping unit 100 may consist of a shaping sleeve having a rectangular cross section, the internal space of which may be connected to the mixing space of the screw kneader of the cylindrical mixer extruder via a graphite bearing 101 having a rectangular cross section. The shaping unit 100 is surrounded by a cooling jacket 98, in which a herical duct is formed for circulating a cooling water 99. Upon passage of the kneaded mixture through the shaping unit 100, it is cooled and solidified to leave a shaped composite product. In the region between the front end bearing 91 of the screw 89 and the graphite bearing 101, there is provided a thermosensor 102 for detecting the temperature of the kneaded composite mixture for serving for maintaining the temperature within a permissible range. The shaping unit 100 can be connected with a transfer means for guiding out the shaped composite product of the metal and the hollow particulate material.

According to the present invention, it is possible to produce, in the first place, a relatively thin, light-weighing composite board of larger surface area in which the particles of the hollow inorganic material are uniformly distributed for use as elements for construction purposes, such as wall board, ceiling, floor board etc. By using Shirasu-balloons as the hollow particulate inorganic material, the present invention can contribute to a development in utilization of useful and economical resources and, by using hollow glass beads, it contributes to a development in the recycled utilization of glass.

In the second place, it is able according to the present invention to obtain relatively thin, non-inflammable light-weighing composite boards of larger surface areas exhibiting a uniform distribution of the material properties for use as construction elements, such as wall boards, ceiling, floor boards and so on, having a voluntarily designed surface profile pattern, whereby the application fields are broadened. By using Shirasu-balloons as the hollow particulate inorganic material, the present invention can participate in a development in the utilization of useful and economical resources and, by using hollow glass beads, it contributes to a development in the recycled utilization of glass. The process according to the present invention is adapted for producing an extended composite board which is in particular suited for producing a high quality composite board having a voluntarily designed surface pattern, since the mold bottom can be composed of a plurality of mold bottom segments connectable with each other into a mold bottom train capable of being forwarded slidingly on a guide way or on a mold bed successively.

In the third place, it is able according to the present invention to obtain composite boards of a metal and a hollow particulate inorganic material, continuously and relatively high thorough-put rate in a vertical material flow, wherein a densely combined composite product is formed continuously by installing a vertically extending passage mold passing through a molten metal storing vessel in the mold cavity of which an aggregation of the particulate inorganic material is forcedly guided downwards successively, wherein a molten metal permeable region of the vertical passage mold which is provided with many small perforations or which is made of a porous refractory material is held immersed in the molten metal layer in the storage vessel so as to permit the molten metal to be injected therethrough into the mold cavity.

In the fourth place, it is able to obtain according to the present invention a light-weighing non-inflammable composite product of a metal and a hollow particulate inorganic material having a uniform distribution of the particles of the inorganic material with a relatively greater bulk thickness adapted for use as a stout element for interior installations in architecture, such as pillars, floor boards, ceiling and so on, by installing a mixer extruder for kneading the molten metal and the hollow particulate inorganic material efficiently and continuously. It brings about many advantages especially in a tall building due to its light-weighing property (a bulk density of less than 1.5 g/cm³). When hollow glass beads (G-light) are used as the hollow particulate material, it can contribute to recycled utilization of glass resources. When Shirasu-balloons, a calcined product of a volcano ejecta deposit, are employed as the hollow particulate material, it participate in development in utilization of useful resources and contributes to a development of new industry.

## Claims

1. A process for producing an extended relatively thin composite product of a metal and a hollow particulate inorganic material using a mold assembly which is constituted essentially of
a mold (13) enclosing a mold cavity (13'') of a geometry corresponding to the extended composite product (17); a means (4, 14) for charging the mold cavity (13'') with the hollow particulate inorganic material; a storage vessel (8) for storing the molten metal; and a means for taking the molded composite product out of the mold cavity (13''),
said process comprising the process steps of
filling up the mold cavity of the mold with the hollow particulate inorganic material to build up an aggregation of the particulate inorganic material in a form corresponding to the mold cavity,
injecting the molten metal into the aggregation of the particulate inorganic material in the mold cavity,
permitting the resulting product composed of the aggregation of the particulate inorganic material and the molten metal to solidify into the extended product of the composite of metal and hollow particulate inorganic material and
taking the solidified composite product out of the mold cavity,
characterized in that
the molten metal is injected through a molten metal permeable perforated or porous refractory plate (13') forming a part of the mold and being located on one side of the extension of the mold cavity (13'') and adjoining to the molten metal in said storage vessel, to cause the molten metal to penetrate into the interstices between the particles in the aggregation by pneumatically impressing the molten metal in the molten metal storage vessel.

2. A process according to claim 1
comprising repeating the process steps of
filling up an entrance section of the mold cavity with the hollow particulate inorganic material to build up an aggregation of the particulate inorganic material therein in a form corresponding to the mold cavity of the entrance section,
forwarding this aggregation slidingly stepwise, first, to a central section of the mold cavity,
injecting the molten metal into the particle aggregation in the central section of the mold cavity through the molten metal permeable perforated or porous refractory plate to cause the molten metal to penetrate the aggregation through the interstices between the particles of said aggregation of the hollow particulate inorganic material by pneumatically impressing the molten metal in the molten metal storage vessel, while re-filling the now vacant entrance section with fresh hollow particulate inorganic material,
forwarding, then, the aggregation found in the central section and now impregnated with the molten metal slidingly stepwise to an exit section of the mold cavity, while repeating the above re-filling and injecting steps,
cooling, thereafter, the resulting molded product in the exit section of the mold cavity to solidify it into the extended product of the composite of metal and hollow particulate inorganic material,
forwarding, then, the aggregations in the three sections slidingly stepwise further to move the solidified product to the outside of the mold, while repeating the above process steps, and
taking the finished molded composite product out of the mold assembly in a discharge station.

3. A process for producing an extended relatively thin product of a composite of a metal and a hollow particulate inorganic material having a voluntarily designed surface relief pattern, successively using a mold assembly constituted essentially of
mold elements (44, 40) enclosing a mold cavity (45) having a profile geometry corresponding to that of the extended product of the composite and composed of, on the one hand, a plurality of mold bottom segments (44) slidably movable on a mold bed (41) and on inlet side and outlet side mold guide ways, respectively, and, on the other hand, a molten metal permeable stationary perforated or porous refractory plate (40); a means (46) for charging the mold cavity (45) with the hollow particulate inorganic material (47); and a storage vessel (35) for storing the molten metal (39), with its bottom being constituted of said molten metal permeable refractory plate (40),
said process comprising, und repetition, the process steps of
laying the mold bottom segments (44) serially on the mold bed (41) to form a mold bed train,
filling up the mold cavity (45) on the mold bottom segment (44) at the mold inlet with the hollow particulate inorganic material to build up an aggregiation of the hollow particulate inorganic material in a form corresponding to the mold cavity,
forwarding the mold bottom train (44) slidingly on the mold guide ways and on the mold bed (41) together with the aggregation of the hollow particulate inorganic material towards the mold outlet,
injecting the molten metal into the mold cavity (45),
taking out the molded extended composite product impregnated wtih the molten metal from the mold bottom segment left the mold as the mold bottom segment moves on, and
removing the foremost mold bottom segment now freed from the molded composite product at the mold outlet end from the outlet side mold guide way and laying it again on the inlet side mold guide way to supplement the mold bottom train,
wherein the molten metal is injected through a molten metal permeable perforated or porous refractory plate (40) forming a part of the mold preferably the bottom of the metal storing vessel (35) and being located on one side of the extension of the mold cavity (45) and adjoining to the molten metal in said storage vessel, to cause the molten metal to penetrate into the interstices between the particles in the aggregation by pneumatically impressing the molten metal in the molten metal storage vessel (35).

4. A process for producing an extended product of a composite of a metal and a hollow particulate inorganic material in a form of a board, cylinder or block, in a continuous way with continuous charging of the hollow particulate inorganic material using a mold assembly constituted essentially of
a stationary passage mold (69) enclosing an extended mold cavity (70) and subdivided into a preheating zone accommodated in a molten metal storage vessel (71), a molten metal injection zone, immersed in the molten metal for permitting injection of the molten metal into the mold cavity (70) therethrough and a cooling zone in the mold exit end portion; an assembly for charging the mold cavity (70) with said hollow particulate inorganic material at the mold inlet; and a towing means for pulling down the resulting extended composite product to be discharged out of the mold,
said process comprising the steps of
charging the mold cavity (70) at the mold inlet with the hollow particulate inorganic material to build up an aggregation of the particulate inorganic material in a cross-sectional profile corresponding to that of the mold cavity (70),
forwarding the resulting aggregation of the particulate inorganic material slidingly towards the mold exit by the action of the towing means,
injecting the molten metal into the mold cavity (70) through a molten metal permeable perforated or porous part of the passage mold (69) through perforations or pore channels being distributed over it to cause the molten metal to penetrate the aggregation of the hollow particulate inorganic material though the interstices between the particles of the aggregation by a static pressure head of the molten metal in the molten metal storage vessel (71) and, if necessary, under a pneumatic pressure control in the molten metal storage vessel (71),
cooling the aggregation impregnated with the molten metal in the cooling zone of the stationary mold (69) to solidify it and
taking the so-solidified extended composite product out of the mold (69) under the use of the towing means.

5. Apparatus for producing an extended composite product of a metal and a hollow particulate inorganic material, comprising
a mold assembly which comprises
a mold (13; 44, 40; 69) enclosing a mold cavity (13''; 45; 70);
a means (4, 14; 46; 63, 64, 67) for charging the mold cavity (13'', 45, 70) with the hollow particulate inorganic material and to shape it into an aggregation (16) of the hollow particulate inorganic material;
a means (11, 20) for forwarding the aggregation (16) of the hollow particulate inorganic material;
a storage vessel (8; 35; 71) for storing the molten metal and adapted to be pneumatically impressed for effecting injection of the molten metal into the mold cavity (13''; 45; 70);
a means (18, 20, 21; 76, 80) for taking the molded composite product (17) out of the mold cavity (13''; 45; 70);
characterized in that a molten metal permeable perforated or porous refractory plate (13') is provided forming part of the mold (13; 44, 40; 69) for injecting the molten metal therethrough into the aggregation (16) of the hollow particulate inorganic material in the mold cavity (13''; 45; 70) with its molten metal permeable perforations (12) or pore channels being distributed over the plate and each having a diameter adapted to permit the molten metal to be injected therethrough into the aggregation (16) upon the pneumatic impression but not adapted to permit the hollow particles of the inorganic material in the aggregation to intrude into the molten metal (10) in said storage vessel (8; 35; 71).

6. Apparatus according to claim 5 for producing an extended relatively thin composite product
characterized in that
the mold (13) encloses a mold cavity (13'') of a geometry corresponding to that of the extended composite product (17),
the means (4, 14) for charging the mold cavity (13'') with the hollow particulate inorganic material is adapted to fill it up and to shape it into an aggregation (16) of the hollow particulate inorganic material,
the means (11, 20) is adapted to slidingly forward the aggregation of the hollow particulate inorganic material from the charging end to a discharge station of the mold assembly,
the refractory plate (13') is located on one side of the extension of the mold cavity and adjoining to the molten metal (10) in said storage vessel (8).

7. Apparatus according to claim 5 for producing and extended relatively thin composite product of a metal and a hollow particulate inorganic material in a continuous way,
characterized in that
the mold (13) encloses a mold cavity (13'') which is subdivided at an equal interval into an entrance section, a central section and an exit section each having the same profile geometry as that of the extended product (17),
the means (4, 14) is adapted to charge the entrance section of the mold cavity (13'') with the hollow particulate inorganic material to fill it up and to build up an aggregation (16) of the hollow particulate inorganic material therein,
the means (11, 20) is adapted for slidingly forwarding stepwise the aggregation of the hollow particulate inorganic material in the entrance section successively to the central and the exit sections of the mold cavity (13'') and, finally, to a discharge station of the mold assembly,
the storage vessel (8) for storing the molten material is located adjacent the mold cavity (13'') and adapted to be pneumatically impressed for effecting injection of the molten metal into the central section of the mold cavity (13''),
the refractory plate (13') is disposed on one side of the extension of the mold cavity (13''),
the means (18, 20, 21) for taking the molded composite product (17) out of the mold cavity (13'') is located at the discharge station.

8. Apparatus according to one of claims 6 or 7, wherein the mold cavity (13'') is defined by a pair of slidable stopper members (14, 21) inserted in a guide path within the mold (13) and movable in synchronism with each other and wherein the pair of slidable stopper members (14, 21) serves as the means for slidingly forwarding the aggregation.

9. Apparatus according to one of claims 6 or 7, wherein the pair of slidable stopper members (14, 18) is composed of a pusher plate (14) and a towing plate (21) having a dovetail recess (18) designed to be disengageable from the solidified molded composite product (17).

10. Apparatus according to one of claims 6 or 7, wherein the storage vessel (8) for the molten metal is a crucible furnace (5) fitted with a gas-tight lid (2) to which is connected a compression gas feed line for effecting the pneumatic impression of the molten metal.

11. Apparatus according to claim 5, for producing an extended relatively thin product of a composite of a metal and a hollow particulate inorganic material having a voluntarily designed surface relief pattern successively, comprising a mold assembly,
characterized in that
mold elements (44, 40) enclose a mold cavity (45) having a profile geometry corresponding to that of the extended product of the composite and composed of a plurality of mold bottom segments (44), which are arranged in a tight but separable fitting with each other to build up a trough-formed mold bottom slidable on a mold bed (41) and on mold guide ways subsequent to and continuing to the mold bed, respectively, and each of which has a voluntarily designed surface relief pattern on the upper face thereof, and a molten metal permeable stationary perforated or porous refractory plate (40) defining the upper limit of the mold cavity (45),
the means (48, 49; 50, 51) is adapted for forwarding the mold bottom slidingly on the mold guide ways and on the mold bed (41) together with said aggregation of the particulate inorganic material carried thereon from the inlet side to the outlet side of the mold assembly,
the storage vessel (35) for storing the molten metal is disposed on the molten metal permeable stationary perforated or porous refractory plate (40),
the means (18, 20, 21) is adapted for taking out the molded extended composite product from the mold bottom segment moved and left the mold cavity (45) on the mold bed (41).

12. An apparatus according to claim 11, wherein one of said plurality of mold bottom segments (44) is replaced by a solid flat board (43) served as a closure member for blocking up passage of the molten metal through the perforated plate (40) before the start of the operation of the apparatus.

13. An apparatus according to claim 11 or 12, wherein each of said plurality of mold bottom segments (44) is designed to permit to be dis- and re-mounted on and from the mold bed (41), so that the foremost segment dismounted from the mold bed (41) is re-mounted on the charge side of the mold assembly.

14. An apparatus according to either one of claims 11 to 13, wherein a piston/cylinder arrangement (48) is used for the means for forwarding the mold bottom segments.

15. An apparatus according to either one of claims 11 to 14, wherein the mold bottom segments (44) are forwarded on the mold bed (41) at a constant velocity.

16. An apparatus according to claim 14 or 15, wherein a support guide (50) for moving the piston/cylinder arrangement (48) is employed for forwarding the mold bottom segments (44).

17. Apparatus according to claim 5 for producing an extended product of a composite of a metal and a hollow particulate inorganic material in a form of a board, cylinder or block, in a continuous way with continuous charging of the hollow particulate inorganic material,
characterized in that
the mold (69) is an extended stationary passage mold enclosing an extended mold cavity (70) having a cross-sectional profile geometry corresponding to that of the extended product of the composite passing therethrough and subdivided into a preheating zone accommodated in a molten metal storage vessel (71), a molten metal injection zone of molten metal permeable perforated or porous part, with its perforations or pore channels being distributed over this zone, immersed in the molten metal for permitting injection of the molten metal into the mold cavity (70) therethrough and a cooling zone in the mold outlet end portion for cooling and solidifying the molded product in the mold cavity (70),
a towing means (76, 80) is adapted for pulling out the resulting extended composite product from the mold cavity (70), disposed subsequent to the mold outlet.

18. An apparatus as claimed in claim 17, wherein a starting dummy (74) is held inserted slidably in the mold cavity (70) before the start of operation of the apparatus.

19. An apparatus as claimed in claim 17, wherein the assembly for charging the mold cavity (70) comprised a casing (64), a screw accommodated therein and operable to introduce the hollow particulate inorganic material into the mold cavity (70) by being actuated by an electric motor (61) connected to the screw shaft (63) rotatably supported in the casing (64), and a hopper (67) for supplying the hollow particulate inorganic material (68) to the inside of the casing (64).

20. An apparatus according to claim 17, wherein the mold element (69) is cooled in its cooling zone by a cooling means (77, 78).

21. An apparatus according to claim 17, wherein the molten metal storage vessel is a crucible furnace fitted with a gas-tight lid to which is connected a compression gas feed line for effecting the pneumatic impression of the molten metal.

## Patentansprüche

1. Verfahren zur Herstellung eines ausgedehnten, relativ dünnen Verbundprodukts aus einem Metall und einem anorganischen Hohlpartikelmaterial unter Verwendung eines Formaufbaus, welcher im wesentlichen umfaßt:
eine Form (13), die einen Formenhohlraum (13'') umschließt, dessen Geometrie dem ausgedehnten Verbundprodukt (17) entspricht; ein Mittel (4, 14) zum Zuführen von anorganischem Hohlpartikelmaterial zu dem Formenhohlraum (13''); einen Vorratsbehälter (8) zur Bereithaltung der Metallschmelze; und ein Mittel zum Entnehmen des geformten Verbundprodukts aus dem Formenhohlraum (13''),
wobei das Verfahren die folgenden Verfahrensschritte umfaßt:
das Auffüllen des Formenhohlraumes der Form mit dem anorganischen Hohlpartikelmaterial zwecks Ausbildung einer Aggregation des anorganischen Partikelmaterials in einer dem Formenhohlraum entsprechenden Form,
das Einspritzen der Metallschmelze in die in dem Formenhohlraum befindliche Aggregation des anorganischen Partikelmaterials, das Aushärten-lassen des im Entstehen begriffenen Produkts, das aus der Aggregation des
anorganischen Partikelmaterials und der Metallschmelze besteht, zu dem ausgedehnten Produkt aus dem Verbundstoff aus Metall und anorganischem Hohlpartikelmaterial, und
das Entnehmen des ausgeharteten Verbundprodukts aus dem Formenhohlraum,
dadurch gekennzeichnet, daß
die Metallschmelze durch ein metallschmelzedurchlässiges, gelochtes bzw. poröses, feuerfestes Blech (13') eingespritzt wird, das einen Teil der Form bildet und an einer Seitenausdehnung des Formenhohlraums (13'') unmittelbar angrenzend an die in dem Vorratsbehälter befindliche Metallschmelze gelegen ist, wobei durch eine pneumatische Druckbeaufschlagung der in dem Metallschmelze-Vorratsbehälter befindlichen Metallschmelze diese Metallschmelze in die Partikelzwischenräume der Aggregation hineingepreßt wird.

2. Verfahren nach Anspruch 1
umfassend die folgenden, sich wiederholenden Verfahrensschritte:
das Auffüllen des Eingangsbereichs des Formenhohlraums mit dem anorganischen Hohlpartikelmaterial, um darin eine Aggregation des anorganischen Partikelmaterials gemäß einer Form auszubilden, welche dem Formenhohlraum des Eingangsbereichs entspricht,
das gleitende, schrittweise Weiterbefördern dieser Aggregation vorerst in den Zentralbereich des Formenhohlraums,
das im Zentralbereich des Formenhohlraums erfolgende Einspritzen der Metallschmelze in die Partikelaggregation durch das metallschmelzedurchlässige, gelochte bzw. poröse, feuerfeste Blech, wobei durch pneumatische Druckbeaufschlagung der in dem Metallschmelze-Vorratsbehälter befindlichen Metallschmelze diese Metallschmelze über die Partikelzwischenräume der Aggregation des anorganischen Hohlpartikelmaterials in diese Aggregation hineingepreßt wird, während der nunmehr freie Eingangsbereich mit neuem, anorganischem Hohlpartikelmaterial befüllt wird,
das anschließend stattfindende, schrittweise, gleitende Weiterbefördern der in dem Zentralbereich befindlichen und nun von der Metallschmelze durchdrungenen Aggregation zu dem Ausgangsbereich des Formenhohlraums, während die oben erwähnten Schritte des Wiederbefüllens und des Einspritzens wiederholt werden,
das daraufhin erfolgende Abkühlen des auf diese Weise geformten Produkts im Ausgangsbereich des Formenhohlraums, in welchem es zu dem ausgedehnten Produkt aus einem Verbundstoff aus Metall und anorganischem Hohlpartikelmaterial ausgehärtet wird,
das anschließend erfolgende, gleitende und schrittweise Weiterbefördern der in den drei Bereichen befindlichen Aggregationen, um das fertig ausgehärtete Produkt aus der Form zu entfernen, während die oben erwähnten Verfahrensschritte wiederholt werden, und
das Entnehmen des fertig geformten Verbundprodukts aus dem Formaufbau im Bereich einer Ablagestation.

3. Verfahren zur Herstellung eines ausgedehnten, relativ dünnen Produkts aus einem Verbundstoff aus Metall und einem anorganischen Hohlpartikelmaterial mit einem beliebig gestalteten Oberflächen-Reliefmuster durch die schrittweise Verwendung eines Formaufbaus, der im wesentlichen die folgenden Elemente umfaßt:
Formelemente (44, 40), welche einen Formenhohlraum (45) mit einer Profilgeometrie umschließen, die jener des ausgedehnten Produkts aus Verbundstoff entspricht, und welche sich einerseits aus einer Vielzahl von Form-Bodensegmenten (44) zusammensetzen, die gleitend beweglich auf einem Formbett (41) bzw. im Form-Eingangsbereich und im Form-Ausgangsbereich jeweils auf einer Formführung angeordnet sind, sowie aus einem stationär angeordneten, metallschmelzedurchlässigen, gelochten bzw. porösen, feuerfesten Blech (40); ein Mittel (46) zum Zuführen von anorganischem Hohlpartikelmaterial (47) zu dem Formenhohlraum (45); und einen Vorratsbehälter (35) zur Bereithaltung der Metallschmelze (39), dessen Boden von dem metallschmelzedurchlässigen, gelochten bzw. porösen, feuerfesten Blech (40) gebildet wird,
wobei das Verfahren die folgenden, sich wiederholenden Verfahrensschritte umfaßt:
das Einlegen der Form-Bodensegmente (44) hintereinander in das Formbett (41), um ein verfahrbares Formbett zu bilden,
das im Eingangsbereich der Form am Form-Bodensegment (44) beginnende Auffüllen des Formenhohlraums (45) mit dem anorganischen Hohlpartikelmaterial, um darin eine der Gestalt des Formenhohlraums entsprechende Aggregation des anorganischen Partikelmaterials auszubilden,
das gleitende Weiterbefördern des verfahrbaren Formbodens (44) auf den Form-Führungsbahnen und auf dem Formbett (41) zusammen mit der Aggregation des anorganischen Hohlpartikelmaterials in Richtung des Formausgangs,
das Einspritzen der Metallschmelze in den Formenhohlraum (45),
das Entnehmen des metallschmelzedurchdrungenen geformten, ausgedehnten Verbundprodukts aus dem links von der Form befindlichen Form-Bodensegment, wahrend der Formboden sich weiterbewegt, und
das im Ausgangsbereich der Form erfolgende Entfernen des nunmehr von dem geformten Verbundprodukt befreiten, vorderen Form-Bodensegments, von der ausgangsseitigen Form-Führungsbahn und dessen erneutes Einlegen in die eingangsseitige Form-Führungsbahn, um den verfahrbaren Formboden wieder zu ergänzen,
wobei die Metallschmelze durch ein metallschmelzedurchlässiges, gelochtes bzw. poröses, feuerfestes Blech (40) hindurch, welches einen Teil der Form, vorzugsweise den Boden des Metall-Vorratsbehälters (35), bildet und an einer Seitenausdehnung des Formenhohlraums (45) unmittelbar angrenzend an die in dem Vorratsbehälter befindliche Metallschmelze angeordnet ist, mittels pneumatischer Druckbeaufschlagung der in dem Vorratsbehälter (35) befindlichen Metallschmelze in die Partikelzwischenräume der Aggregation hineingepreßt wird.

4. Verfahren zur kontinuierlichen Herstellung eines ausgedehnten Produkts aus einem Verbundstoff aus Metall und anorganischem Hohlpartikelmaterial in der Form einer Platte, eines Zylinders oder eines Blocks durch eine kontinuierliche Befüllung mit dem anorganischen Hohlpartikelmaterial unter Verwendung eines Formaufbaus, der im wesentlichen die folgenden Elemente umfaßt:
eine stationäre Durchlaufform (69), die einen ausgedehnten Formenhohlraum (70) umschließt und erstens in einen Vorwärmabschnitt, der an dem Metallschmelze-Vorratsbehälter (71) vorgesehen ist, zweitens in einen Metallschmelze-Einspritzabschnitt, der in die Metallschmelze eingetaucht ist, um ein durch ihn hindurch erfolgendes Einspritzen der Metallschmelze in den Formenhohlraum (70) zu ermöglichen, und drittens in einen im Form-Ausgangsbereich angeordneten Kühlabschnitt unterteilt ist; eine am Form-Eingang angeordnete Vorrichtung zum Zuführen des anorganischen Hohlpartikelmaterials zu dem Formenhohlraum (70); und ein Schleppmittel zum Herabziehen des auf diese Weise geformten, ausgedehnten Verbundprodukts, das aus der Form zu entnehmen ist,
wobei das Verfahren die folgenden Verfahrensschritte umfaßt:
das am Form-Eingang stattfindende Befüllen des Formenhohlraums (70) mit dem anorganischen Hohlpartikelmaterial zwecks Ausbildung einer Aggregation des anorganischen Hohlpartikelmaterials gemäß einem Querschnittprofil, das jenem des Formenhohlraums (70) entspricht,
das von den Schleppmitteln angetriebene, gleitende Weiterbefördern der auf diese Weise gewonnenen Aggregation des anorganischen Partikelmaterials in Richtung des Form-Ausgangs,
das Einspritzen der Metallschmelze in den Formenhohlraum (70) über den metallschmelzedurchlässigen, gelochten bzw. porösen Bereich der Durchlaufform (69) durch die über dessen Oberfläche hinweg verteilten Öffnungen bzw. Porenkanäle, wobei die Metallschmelze infolge eines statischen Druckgefälles der in dem Metallschmelze-Vorratsbehälter (71) befindlichen Metallschmelze und, sofern erforderlich, durch eine pneumatische Druckregelung des Metallschmelze-Vorratsbehälters (71) die Aggregation des anorganischen Hohlpartikelmaterials durchdringt und deren Partikelzwischenräume auffüllt,
das in dem Kühlabschnitt der stationären Form (69) erfolgende Abkühlen und Aushärten des von der Metallschmelze durchdrungenen Aggregats, und
das unter Verwendung der Schleppmittel vor sich gehende Entnehmen des auf diese Weise ausgehärteten, ausgedehnten Verbundprodukts aus der Form (69).

5. Vorrichtung zur Herstellung eines ausgedehnten Verbundprodukts aus einem Metall und einem anorganischen Hohlpartikelmaterial, umfassend
einen Formaufbau, welcher folgendes umfaßt:
eine Form (13; 44, 40; 69), welche einen Formenhohlraum (13''; 45; 70) umschließt;
ein Mittel (4, 14; 46; 63, 64, 67) zum Zuführen von anorganischem Hohlpartikelmaterial zu dem Formenhohlraum (13'', 45, 70) und zum Ausbilden einer Aggregation (16) des anorganischen Hohlpartikelmaterials;
ein Mittel (16, 20) zum Weiterbefördern der Aggregation (16) des anorganischen Hohlpartikelmaterials;
einen Vorratsbehälter (8; 35; 71) zur Bereithaltung der Metallschmelze, welcher zum Zweck der Einspritzung der Metallschmelze in den Formenhohlraum (13''; 45; 70) mit pneumatischem Druck beaufschlagt werden kann;
ein Mittel (18, 20, 21; 76, 80) zum Entnehmen des geformten Verbundprodukts (17) aus dem Formenhohlraum (13''; 45; 70);
dadurch gekennzeichnet, daß als Bestandteil der Form (13; 44, 40; 69) ein metallschmelzedurchlässiges, gelochtes bzw. poröses, feuerfestes Blech (13') vorgesehen ist, durch welches hindurch die Metallschmelze in die in dem Formenhohlraum (13''; 45; 70) befindliche Aggregation (16) des anorganisches Hohlpartikelmaterials eingespritzt werden kann, wobei dessen metallschmelzedurchlässige Öffnungen (12) bzw. Porenkanäle über das Blech hinweg verteilt angeordnet sind und ihre Durchmesser jeweils entsprechend bemessen sind, daß die Metallschmelze bei pneumatischer Druckbeaufschlagung des Behälters durch sie hindurch in die Aggregation (16) eingespritzt werden kann, daß jedoch umgekehrt ein Eindringen der Hohlpartikel des anorganischen Materials in die in dem Vorratsbehälter (8; 35; 71) befindliche Metallschmelze (10) verhindert wird.

6. Vorrichtung zur Herstellung eines ausgedehnten, relativ dünnen Verbundprodukts nach Anspruch 5,
dadurch gekennzeichnet, daß
die Form (13) einen Formenhohlraum (13'') umschließt, dessen Geometrie jener des ausgedehnten Verbundprodukts (17) entspricht,
das Mittel (4, 14) zum Zuführen des anorganischen Hohlpartikelmaterials zu dem Formenhohlraum (13'') dazu geeignet ist, diesen aufzufüllen und darin eine Aggregation (16) des anorganischen Hohlpartikelmaterials auszubilden,
das Mittel (11, 20) dazu geeignet ist, die Aggregation des anorganischen Hohlpartikelmaterials in gleitender Weise von dem Zuführbereich bis zu der Entnahmestation des Formaufbaus weiterzubefördern,
das feuerfeste Blech (13') an einer Seitenausdehnung des Formenhohlraums unmittelbar angrenzend an die in dem Vorratsbehälter (8) befindliche Metallschmelze (10) angeordnet ist.

7. Vorrichtung zur kontinuierlichen Herstellung eines ausgedehnten, relativ dünnen Verbundprodukts aus einem Metall und einem anorganischen Hohlpartikelmaterial,
dadurch gekennzeichnet, daß
die Form (13) einen Formenhohlraum (13'') umschließt, welcher in gleichen Intervallen in einen Eingangsbereich, einen Zentralbereich und einen Ausgangsbereich unterteilt ist, und von denen ein jeder über dieselbe Geometrie verfügt wie das ausgedehnte Produkt (17),
das Mittel (4, 14) dazu geeignet ist, das anorganische Hohlpartikelmaterial dem Eingangsbereich des Formenhohlraumes (13'') zuzuführen, diesen damit zu befüllen und darin eine Aggregation (16) des anorganischen Hohlpartikelmaterials auszubilden,
das Mittel (11, 20) dazu geeignet ist, die auf diese Weise im Eingangsbereich bereitgestellte Aggregation des anorganischen Hohlpartikelmaterials in gleitender Weise der Reihe nach zum Zentralbereich und zum Ausgangsbereich des Formenhohlraums (13''), und schließlich zu der Ablagestation des Formaufbaus weiterzubefördern,
der Vorratsbehälter (8) zum Bereithalten der Metallschmelze unmittelbar angrenzend an den Formenhohlraum (13'') angeordnet ist und zum Zweck der Einspritzung der Metallschmelze in den Zentralbereich des Formenhohlraums (13'') mit pneumatischem Druck beaufschlagt werden kann,
das feuerfeste Blech (13') an einer Seitenausdehnung des Formenhohlraums (13'') angeordnet ist,
das Mittel (18, 20, 21) zum Entnehmen des geformten Verbundprodukts (17) aus dem Formenhohlraum (13'') im Bereich der Ablagestation angeordnet ist.

8. Vorrichtung nach einem der Ansprüche 6 oder 7, wobei der Formenhohlraum (13'') von einem Paar gleitend verschiebbarer Schließelemente (14, 21) definiert wird, die in die Führungsbahn innerhalb der Form (13) eingesetzt werden und synchron zueinander beweglich sind, und wobei dieses Paar gleitend verschiebbarer Schließelemente (14, 21) als Mittel zum gleitenden Weiterbefördern der Aggregation dient.

9. Vorrichtung nach einem der Ansprüche 6 oder 7, wobei das Paar gleitend verschiebbarer Schließelemente (14, 18) aus einem Schiebeblech (14) und einem Ziehblech (21) besteht, von denen letzteres über eine schwalbenschwanzförmige Ausnehmung (18) verfügt, welche entsprechend ausgebildet ist, um von dem ausgehärteten, geformten Verbundprodukt (17) abgenommen werden zu können.

10. Vorrichtung nach einem der Ansprüche 6 oder 7, wobei es sich bei dem Metallschmelze-Vorratsbehälter (8) um einen Tiegelschmelzofen (5) handelt, welcher mit einem gasdichten Deckel (2) ausgestattet ist, an dem zum Zweck der pneumatischen Druckbeaufschlagung der Metallschmelze eine Druckgas-Zuführleitung angebracht ist.

11. Vorrichtung nach Anspruch 5 zur aufeinanderfolgenden Herstellung eines ausgedehnten, relativ dünnen Produkts aus einem Verbundstoff aus Metall und anorganischem Hohlpartikelmaterial mit einem beliebig gestalteten Oberflächen-Reliefmuster, deren Formaufbau
dadurch gekennzeichnet ist, daß
die Formelemente (44, 40) einen Formenhohlraum (45) mit einer Profilgeometrie umschließen, die jener des ausgedehnten Verbundprodukts entspricht, und der sich aus einer Vielzahl von Form-Bodensegmenten (44) zusammensetzt, welche in einer festen jedoch trennbaren Verbindung zueinander stehen und einen verfahrbaren, trogförmigen Formboden bilden, der gleitend beweglich auf einem Formbett (41) und auf daran anschließende und dieses fortsetzende Form-Führungsbahnen angeordnet ist, wobei ein jedes von ihnen an seiner Oberseite über ein beliebig gestaltetes Oberflächen-Reliefmuster verfügt, sowie weiters ein metallschmelzedurchlässiges, stationär angeordnetes, gelochtes bzw. poröses, feuerfestes Blech (40) aufweist, welches die obere Begrenzung des Formenhohlraums (45) darstellt,
das Mittel (48, 49; 50, 51) dazu geeignet ist, den Formboden in gleitender Weise auf den Form-Führungsbahnen und auf dem Formbett (41) zusammen mit der darauf transportierten Aggregation des anorganischen Partikelmaterials von der Eingangsseite zu der Ausgangsseite des Formaufbaus weiterzubefördern,
der Vorratsbehälter (35) zur Bereithaltung der Metallschmelze auf dem metallschmelzedurchlässigen, stationären, gelochten bzw. porösen, feuerfesten Blech (40) angebracht ist,
das Mittel (18, 20, 21) dazu geeignet ist, das geformte, ausgedehnte Verbundprodukt aus dem Form-Bodensegment zu entnehmen, sobald dieses sich weiterbewegt und den Formenhohlraum (45) auf dem Formbett (41) verlassen hat.

12. Vorrichtung nach Anspruch 11, wobei eines der Form-Bodensegmente (44) durch ein flaches Vollblech (43) ersetzt wird, das als Verschlußelement dient und ein vorzeitiges Ausfließen der Metallschmelze durch das gelochte Blech (40) vor dem Fertigungsbeginn verhindert.

13. Vorrichtung nach Anspruch 11 oder 12, wobei ein jedes der Form-Bodensegmente (44) getrennt auf das Formbett (41) auf- bzw. wieder von diesem abmontierbar ist, sodaß das vorderste Segment von dem Formbett (41) abmontiert werden kann und auf der Zuführseite zu dem Formaufbau wieder aufmontiert werden kann.

14. Vorrichtung nach einem der Ansprüche 11 bis 13, wobei als Mittel zum Weiterbefördern der Form-Bodensegmente eine Preßkolben/Zylinder-Einrichtung (48) verwendet wird.

15. Vorrichtung nach einem der Ansprüche 11 bis 14, wobei die Form-Bodensegmente (44) mit konstanter Geschwindigkeit aufdem Formbett (41) weiterbefördert werden.

16. Vorrichtung nach Anspruch 14 oder 15, wobei eine Führungsrille (50) zum Einsatz kommt, in der sich die Preßkolben/Zylindereinrichtung (48) beim Weiterbefördern der Form-Bodensegmente (44) bewegt.

17. Vorrichtung nach Anspruch 5 zur kontinuierlichen Herstellung eines ausgedehnten Produkts aus einem Verbundstoff aus Metall und anorganischem Hohlpartikelmaterial in der Form einer Platte, eines Zylinders oder eines Blocks unter kontinuierlicher Zuführung des anorganischen Hohlpartikelmaterials,
dadurch gekennzeichnet, daß
es sich bei der Form (69) um eine ausgedehnte, stationäre Durchlaufform handelt, welche einen ausgedehnten Formenhohlraum (70) umschließt, dessen Querschnittprofilgeometrie jener des ausgedehnten, diesen Formenhohlraum durchlaufenden Verbundprodukts entspricht, und welche erstens in einen Vorwärmabschnitt, der an einem Metallschmelze-Vorratsbehälter (71) vorgesehen ist, zweitens in einen Metallschmelze-Einspritzabschnitt mit einem metallschmelzedurchlässigen, gelochten bzw. porösen Bereich, dessen Öffnungen bzw. Porenkanäle über diesen Bereich hinweg verteilt sind und der in die Metallschmelze eingetaucht ist, um ein Einspritzen der Metallschmelze in den Formenhohlraum (70) durch diesen hindurch zu ermöglichen, und drittens in einen im Form-Ausgangsbereich angeordneten Kühlabschnitt zum Abkühlen und Aushärten des in dem Formenhohlraum (70) befindlichen, geformten Produkts unterteilt ist,
das im Anschluß an den Form-Ausgang angeordnete Schleppmittel (76, 80) dazu geeignet ist, das auf diese Weise geformte, ausgedehnte Verbundprodukt aus dem Formenhohlraum (70) zu entnehmen.

18. Vorrichtung gemäß Anspruch 17, wobei vor Aufnahme des Betriebs der Vorrichtung ein Anfahrsegment (74) in gleitender Weise in den Formenhohlraum (70) eingeführt und darin festgehalten wird.

19. Vorrichtung gemäß Anspruch 17, wobei die Einrichtung zum Befüllen des Formenhohlraums (70) aus einem Gehäuse (64), einer darin vorgesehenen Schnecke, durch deren Drehung das anorganische Hohlpartikelmaterial in den Formenhohlraum (70) eingebracht wird und die von einem Elektromotor (61) angetrieben wird, welcher mit der drehbar in dem Lager (64) gelagerten Schneckenwelle (63) verbunden ist, sowie aus einem Magazin (67) zum Einbringen des anorganischen Hohlpartikelmaterials (68) in das Innere des Gehäuses (64) besteht.

20. Vorrichtung gemäß Anspruch 17, wobei das Formelement (69) im Bereich seines Kühlabschnitts durch eine Kühleinrichtung (77, 78) abgekühlt wird.

21. Vorrichtung gemäß Anspruch 17, wobei es sich bei dem Metallschmelze-Vorratsbehälter um einen Tiegelschmelzofen handelt, der mit einem gasdichten Deckel ausgestattet ist, an dem zum Zweck der pneumatischen Druckbeaufschlagung der Metallschmelze eine Druckgas-Zuführleitung angebracht ist.

## Revendications

1. Procédé de fabrication d'un produit composite étendu relativement mince fait d'un métal et d'un matériau minéral particulaire creux, utilisant un ensemble de moule qui est constitué essentiellement
d'un moule (13) enfermant une cavité de moule (13'') dont la géométrie correspond au produit composite étendu (17) ; d'un moyen (4, 14) destiné à charger la cavité de moule (13'') avec le matériau minéral particulaire creux ; d'un réservoir de stockage (8) destiné à stocker le métal fondu ; et d'un moyen destiné à prélever le produit composite moulé hors de la cavité du moule (13''),
ledit procédé comprenant les étapes de procédé consistant à
remplir la cavité de moule du moule avec le matériau minéral particulaire creux afin d'accumuler une agrégation du matériau minéral particulaire sous une forme qui correspond à la cavité du moule,
injecter le métal fondu dans l'agrégation du matériau minéral particulaire dans la cavité du moule,
permettre que le produit résultant composé de l'agrégation du matériau minéral particulaire et du métal fondu se solidifie dans le produit étendu du composite du métal et du matériau minéral particulaire creux, et
prélever le produit composite solidifié hors de la cavité du moule,
caractérisé en ce que
le métal fondu est injecté au travers d'une plaque réfractaire perforée ou poreuse perméable au métal fondu (13') formant une partie du moule qui est située d'un côté de l'extension de la cavité du moule (13'') et contiguë au métal fondu dans ledit réservoir de stockage, afin d'amener le métal fondu à pénétrer jusque dans les interstices entre les particules de l'agrégation en pressant pneumatiquement le métal fondu dans le réservoir de stockage de métal fondu.

2. Procédé selon la revendication 1 comprenant la répétition des étapes de procédé consistant à
remplir une section d'entrée de la cavité du moule avec le matériau minéral particulaire creux afin d'accumuler une agrégation du matériau minéral particulaire dans celle-ci suivant une forme correspondant à la cavité de moule de la section d'entrée,
faire avancer pas à pas par glissement cette agrégation, tout d'abord, vers une section centrale de la cavité du moule,
injecter le métal fondu jusque dans l'agrégation de particules dans la section centrale de la cavité du moule par l'intermédiaire de la plaque réfractaire perforée ou poreuse perméable au métal fondu, afin d'amener le métal fondu à pénétrer dans l'agrégation au travers des interstices entre les particules de ladite agrégation du matériau minéral particulaire creux en pressant pneumatiquement le métal fondu dans le réservoir de stockage de métal fondu, tout en remplissant à nouveau la section d'entrée maintenant vide avec un nouveau matériau minéral particulaire creux,
faire alors avancer l'agrégation qui se trouve dans la section centrale et qui est maintenant imprégnée du métal fondu, pas à pas par glissement vers une section de sortie de la cavité du moule, tout en répétant les étapes précitées de nouveau remplissage et d'injection,
refroidir, ensuite, le produit moulé résultant dans la section de sortie de la cavité du moule, afin de le solidifier en le produit étendu du composite de métal et de matériau minéral particulaire creux,
faire alors avancer les agrégations davantage dans les trois sections pas à pas par glissement, afin de déplacer le produit solidifié vers l'extérieur du moule, tout en répétant les étapes du procédé ci-dessus, et
prélever le produit composite moulé terminé hors de l'ensemble de moule dans un poste de déchargement.

3. Procédé de fabrication d'un produit mince relativement étendu d'un composite d'un métal et d'un matériau minéral particulaire creux comportant un motif en relief de surface volontairement conçu, en utilisant successivement un ensemble de moule constitué essentiellement
d'éléments de moule (44, 40) enfermant une cavité de moule (45) présentant une géométrie de profil correspondant à celle du produit étendu du composite et composée, d'une part, d'une pluralité de segments de fond de moule (44) mobiles par glissement sur un lit de moule (41) et sur des voies de guidage de moule du côté de l'orifice d'entrée et du côté de l'orifice de sortie, respectivement, et, d'autre part, d'une plaque réfractaire perforée ou poreuse immobile, perméable au métal fondu (40) ; d'un moyen (46) destiné à charger la cavité du moule (45) avec le matériau minéral particulaire creux (47) ; et d'un réservoir de stockage (35) destiné à stocker le métal fondu (39), dont le fond est constitué de ladite plaque réfractaire perméable au métal fondu (40),
ledit procédé comprenant, en répétition, les étapes de procédé consistant à
déposer les segments de fond de moule (44) en série sur le lit de moule (41) afin de former un train de lit de moule,
remplir la cavité du moule (45) sur le segment de fond de moule (44) au niveau de l'orifice d'entrée de moule avec le matériau minéral particulaire creux, afin d'accumuler une agrégation du matériau minéral particulaire creux sous une forme correspondant à la cavité du moule,
faire avancer le train de fond de moule (44) par glissement sur les voies de guidage de moule et sur le lit de moule (41) en même temps que l'agrégation du matériau minéral particulaire creux en direction de l'orifice de sortie du moule,
injecter le métal fondu jusque dans la cavité du moule (45),
prélever le produit composite étendu moulé imprégné du métal fondu depuis le segment de fond de moule qui a quitté le moule lorsque le segment de fond de moule se déplace, et
enlever le segment de fond de moule le plus en avant maintenant libéré du produit composite moulé au niveau de l'extrémité de l'orifice de sortie de moule depuis la voie de guidage de moule du côté orifice de sortie, et le déposer à nouveau sur la voie de guidage de moule du côté orifice d'entrée afin de compléter le train de fond de moule,
procédé dans lequel le métal fondu est injecté au travers d'une plaque réfractaire perforée ou poreuse perméable au métal fondu (40) formant une partie du moule, de préférence le fond du réservoir de stockage de métal (35), et étant située sur un côté de l'extension de la cavité de moule (45) et contiguë au métal fondu dans ledit réservoir de stockage, afin d'amener le métal fondu à pénétrer jusque dans les interstices entre les particules de l'agrégation en pressant pneumatiquement le métal fondu dans le réservoir de stockage de métal fondu (35).

4. Procédé de fabrication en continu d'un produit étendu d'un composite d'un métal et d'un matériau minéral particulaire creux sous forme d'une plaque, d'un cylindre ou d'un bloc, avec un chargement en continu du matériau minéral particulaire creux, utilisant un ensemble de moule constitué essentiellement
d'un moule de passage immobile (69) enfermant une cavité de moule étendue (70) et subdivisé en une zone de préchauffage logée dans un réservoir de stockage de métal fondu (71), une zone d'injection de métal fondu, immergée dans le métal fondu afin de permettre l'injection du métal fondu jusque dans la cavité du moule (70) au travers de celle-ci, et une zone de refroidissement dans la partie d'extrémité de sortie du moule ; d'un ensemble destiné à charger la cavité du moule (70) avec ledit matériau minéral particulaire creux au niveau de l'orifice d'entrée du moule; et d'un moyen de tirage destiné à sortir le produit composite étendu résultant devant être déchargé du moule,
ledit procédé comprenant les étapes consistant à
charger la cavité du moule (70) au niveau de l'orifice d'entrée du moule avec le matériau minéral particulaire creux afin d'accumuler une agrégation du matériau minéral particulaire dans un profil correspondant en section transversale à celui de la cavité du moule (70),
faire avancer l'agrégation résultante du matériau minéral particulaire par glissement en direction de la sortie du moule grâce à l'action du moyen de tirage,
injecter le métal fondu jusque dans la cavité du moule (70) par l'intermédiaire d'une partie perforée ou poreuse perméable au métal fondu du moule de passage (69) au travers de perforations ou de canaux de pores qui sont répartis sur celle-ci, afin d'amener le métal fondu à pénétrer dans l'agrégation du matériau minéral particulaire creux au travers des interstices entre les particules de l'agrégation grâce à une différence de pression statique du métal fondu dans le réservoir de stockage de métal fondu (71) et, si nécessaire, sous une commande de pression pneumatique dans le réservoir de stockage de métal fondu (71),
refroidir l'agrégation imprégnée du métal fondu dans la zone de refroidissement du moule immobile (69) afin de la solidifier et
prélever le produit composite étendu ainsi solidifié hors du moule (69) par l'utilisation du moyen de traction.

5. Dispositif destiné à fabriquer un produit composite étendu d'un métal et d'un matériau minéral particulaire creux, comprenant
un ensemble de moule qui comprend
un moule (13 ; 44, 40 ; 69) enfermant une cavité de moule (13'' ; 45 ; 70),
un moyen (4, 14 ; 46 ; 63, 64, 67) destiné à charger la cavité du moule (13'' ; 45 ; 70) avec le matériau minéral particulaire creux et à le mettre sous la forme d'une agrégation (16) du matériau minéral particulaire creux,
un moyen (11, 20) destiné à faire avancer l'agrégation (16) du matériau minéral particulaire creux,
un réservoir de stockage (8 ; 35 ; 71) destiné à stocker le métal fondu et conçu pour être pressé pneumatiquement afin de réaliser l'injection du métal fondu jusque dans la cavité du moule (13'' ; 45 ; 70),
un moyen (18, 20, 21 ; 76, 80) destiné à prélever le produit composite moulé (17) hors de la cavité du moule (13'' ; 45 ; 70),
caractérisé en ce qu'une plaque réfractaire perforée ou poreuse perméable au métal fondu (13') est prévue comme faisant partie du moule (13 ; 44, 40 ; 69) afin d'injecter le métal fondu au travers de celle-ci jusque dans l'agrégation (16) du matériau minéral particulaire creux dans la cavité du moule (13'' ; 45 ; 70), ses perforations ou canaux de pores perméables au métal fondu (12) étant répartis sur la plaque et présentant chacun un diamètre conçu pour permettre au métal fondu d'être injecté au travers de ceux-ci jusque dans l'agrégation (16) lors de la mise en pression pneumatique, tout en étant conçu pour ne pas permettre aux particules creuses du matériau minéral de l'agrégation de s'introduire jusque dans le métal fondu (10) dans ledit réservoir de stockage (8 ; 35 ; 71).

6. Dispositif selon la revendication 5, destiné à fabriquer un produit composite relativement mince étendu
caractérisé en ce que
le moule (13) enferme une cavité de moule (13'') d'une géométrie qui correspond à celle du produit composite tendu (17),
le moyen (4, 14) destiné à charger la cavité du moule (13'') avec le matériau minéral particulaire creux est agencé pour la remplir et pour le mettre en forme en une agrégation (16) du matériau minéral particulaire creux,
le moyen (11, 20) est agencé pour faire avancer par glissement l'agrégation du matériau minéral particulaire creux depuis l'extrémité de chargement vers un poste de déchargement de l'ensemble de moule,
la plaque réfractaire (13') est située d'un côté de l'extension de la cavité du moule et contiguë au métal fondu (10) dans ledit réservoir de stockage (8).

7. Dispositif selon la revendication 5, destiné à fabriquer en continu un produit composite relativement mince étendu d'un métal et d'un matériau minéral particulaire creux,
caractérisé en ce que
le moule (13) enferme une cavité de moule (13'') qui est subdivisée, avec des intervalles égaux, en une section d'entrée, une section centrale et une section de sortie présentant chacune la même géométrie de profil que celle du produit étendu (17),
le moyen (4, 14) est agencé pour charger la section d'entrée de la cavité du moule (13'') avec le matériau minéral particulaire creux afin de la remplir et d'accumuler une agrégation (16) du matériau minéral particulaire creux dans celle-ci,
le moyen (11, 20) est agencé pour faire avancer par glissement pas à pas l'agrégation du matériau minéral particulaire creux dans la section d'entrée, successivement vers les sections centrale et de sortie de la cavité du moule (13'') et, finalement, vers un poste de déchargement de l'ensemble de moule,
le réservoir de stockage (8) destiné à stocker le matériau fondu est situé de façon contiguë à la cavité du moule (13'') et agencé pour être pressé pneumatiquement afin de réaliser l'injection du métal fondu jusque dans la section centrale de la cavité du moule (13''),
la plaque réfractaire (13') est disposée d'un côté de l'extension de la cavité du moule (13''),
le moyen (18, 20, 21) destiné à prélever le produit composite moulé (17) hors de la cavité du moule (13'') est situé au niveau du poste de déchargement.

8. Dispositif selon l'une des revendications 6 et 7, dans lequel la cavité du moule (13'') est définie par une paire d'éléments de bouchons coulissants (14, 21), insérés dans un chemin de guidage à l'intérieur du moule (13) et mobiles en synchronisme l'un avec l'autre, et dans lequel la paire d'éléments de bouchons coulissants (14, 21) sert de moyen destiné à faire avancer par glissement l'agrégation.

9. Dispositif selon l'une des revendications 6 et 7, dans lequel la paire d'éléments de bouchons coulissants (14, 18) est composée d'une plaque de poussée (14) et d'une plaque de tirage (21) comportant un évidement en queue d'aronde (18) conçue pour pouvoir être dégagée du produit composite moulé solidifié (17).

10. Dispositif selon l'une des revendications 6 et 7, dans lequel le réservoir de stockage (8) destiné au métal fondu est un four à creuset (5) muni d'un couvercle étanche aux gaz (2) auquel est reliée une conduite d'alimentation en gaz de compression destinée à réaliser la mise en pression pneumatique du métal fondu.

11. Dispositif selon la revendication 5, destiné à fabriquer un produit relativement mince étendu d'un composite d'un métal et d'un matériau minéral particulaire creux présentant un motif en relief en surface volontairement conçu, comprenant un ensemble de moule,
caractérisé en ce que
des éléments de moule (44, 40) enferment une cavité de moule (45) présentant une géométrie de profil qui correspond à celle du produit étendu du composite et composée d'une pluralité de segments de fond de moule (44), qui sont agencés suivant un montage serré mais séparable, afin de construire un fond de moule en forme d'auge pouvant coulisser sur un lit de moule (41) et sur des voies de guidage de moule à la suite du lit de moule et le prolongeant, respectivement, et dont chacun présente un motif en relief en surface volontairement conçu sur la face supérieure de celui-ci, et une plaque réfractaire perforée ou poreuse immobile perméable au métal fondu (40) définissant la limite supérieure de la cavité du moule (45),
le moyen (48, 49 ; 50, 51) est conçu pour faire avancer par glissement le fond de moule sur les voies de guidage de moule et sur le lit de moule (41) en même temps que ladite agrégation du matériau minéral particulaire transporté sur celui-ci depuis le côté de l'orifice d'entrée vers le côté de l'orifice de sortie de l'ensemble de moule,
le réservoir de stockage (35) destiné à stocker le métal fondu est disposé sur la plaque réfractaire perforée ou poreuse immobile perméable au métal fondu (40),
le moyen (18, 20, 21) est conçu pour prélever le produit composite étendu moulé depuis le segment de fond de moule déplacé et qui a quitté la cavité de moule (45) sur le lit de moule (41).

12. Dispositif selon la revendication 11, dans lequel un segment de ladite pluralité de segments de fond de moule (44) est remplacé par une plaque plate pleine (43) utilisée en tant qu'élément de fermeture pour le blocage du passage du métal fondu au travers de la plaque perforée (40) avant le début du fonctionnement du dispositif.

13. Dispositif selon la revendication 11 ou 12, dans lequel chaque segment de ladite pluralité de segments de fond de moule (44) est conçu pour permettre qu'il soit démonté du lit de moule (41) et remonté sur celui-ci, de façon à ce que le segment le plus en avant démonté du lit de moule (41) soit remonté sur le côté de chargement de l'ensemble de moule.

14. Dispositif selon l'une quelconque des revendications 11 à 13, dans lequel un agencement de piston/cylindre (48) est utilisé pour le moyen destiné à faire avancer les segments de fond de moule.

15. Dispositif selon l'une quelconque des revendications 11 à 14, dans lequel les segments de fond de moule (44) sont avancés sur le lit de moule (41) à vitesse constante.

16. Dispositif selon la revendication 14 ou 15, dans lequel un guide de support (50) destiné à déplacer l'agencement de piston/cylindre (48) est utilisé pour faire avancer les segments de fond de moule (44).

17. Dispositif selon la revendication 5, destiné à fabriquer en continu un produit étendu d'un composite d'un métal et d'un matériau minéral particulaire creux sous forme d'une plaque, d'un cylindre ou d'un bloc, avec un chargement en continu du matériau minéral particulaire creux,
caractérisé en ce que
le moule (69) est un moule de passage immobile étendu enfermant une cavité de moule étendue (70) présentant une géométrie de profil en section transversale qui correspond à celle du produit étendu du composite passant au travers de celle-ci et subdivisée en une zone de préchauffage logée dans un réservoir de stockage de métal fondu (71), une zone d'injection de métal fondu faite d'une partie perforée ou poreuse perméable au métal fondu, dont les perforations ou les canaux de pores sont répartis sur cette zone, immergée dans le métal fondu afin de permettre l'injection du métal fondu jusque dans la cavité du moule (70) au travers de celle-ci, et une zone de refroidissement dans la partie d'extrémité d'orifice de sortie du moule afin de refroidir et de solidifier le produit moulé dans la cavité du moule (70),
un moyen de tirage (76, 80) est agencé pour sortir le produit composite étendu résultant de la cavité du moule (70), disposé après l'orifice de sortie du moule.

18. Dispositif selon la revendication 17, dans lequel une fausse charge de départ (74) est maintenue insérée de façon glissante dans la cavité du moule (70) avant le début du fonctionnement du dispositif.

19. Dispositif selon la revendication 17, dans lequel l'ensemble destiné au chargement de la cavité du moule (70) comprend un carter (64), une vis logée dans celui-ci et pouvant être mise en oeuvre pour introduire le matériau minéral particulaire creux jusque dans la cavité du moule (70) en étant actionnée par un moteur électrique (61) accouplé à l'axe de la vis (63) supporté avec possibilité de rotation dans le carter (64), et une trémie (67) destinée à alimenter le matériau minéral particulaire creux (68) jusqu'à l'intérieur du carter (64).

20. Dispositif selon la revendication 17, dans lequel l'élément de moule (69) est refroidi dans sa zone de refroidissement par un moyen de refroidissement (77, 78).

21. Dispositif selon la revendication 17, dans lequel le réservoir de stockage de métal fondu est un four à creuset muni d'un couvercle étanche aux gaz, auquel est reliée une conduite d'alimentation en gaz de compression destinée à réaliser la mise en pression pneumatique du métal fondu.
